

# United States Patent Office

2,936,320

Patented May 10, 1960

1

2,936,320

## DIESTERS OF MIXED AROMATIC DIBASIC ACIDS

George J. Benoit, Jr., San Anselmo, Calif., assignor to California Research Corporation, San Francisco, Calif., a corporation of Delaware

No Drawing. Application June 24, 1957  
Serial No. 667,716

4 Claims. (Cl. 260—475)

This invention relates to novel diesters of mixed aromatic dibasic acids. More particularly, the invention is concerned with a new class of dialkyl diesters of mixtures of isophthalic acid and terephthalic acid which are excellent synthetic oils. 15

Synthetic oils are important as lubricants in a variety of applications where there are certain specific requirements not met by the more common lubricating oils such as mineral oils. Applications of this type include the lubrication of instruments, weapons, optical equipment and aircraft gas turbines of the "prop" and "jet" types.

In general, a combination of special properties is desirable in synthetic oils for applications of the above type. Fluidity at low temperatures and low volatility high temperatures are important characteristics. Similarly, good viscosity-temperature characteristics are desirable since proper lubrication in most applications requires that the lubricant be adaptable to changes in temperature without extreme variations in viscosity.

The most critical characteristic of synthetic lubricating oils in the important application to aircraft gas turbines is the resistance of the oil to thermal degradation at high temperatures. Aircraft gas turbines are being operated at increasingly higher temperatures where the formation of coke, due to the thermal decomposition and deterioration of the lubricant, is a major problem. The proper functioning of the lubrication system is impeded by the formation of deposits on bearing cages and housings and the plugging of oil filters.

It has now been found that a superior new class of diesters of mixed aromatic dibasic acids, namely, the dialkyl diesters of mixtures of isophthalic acid and terephthalic acid in which the alkyl esterifying groups are derived from a mixture of aliphatic alcohols of from 5 to 13 carbon atoms each, are excellent synthetic oils having special properties which make them unusually desirable as synthetic lubricants.

The superior new class of dialkyl diesters of mixtures of isophthalic acid and terephthalic acid, according to the present invention as described above, possesses a desirably low volatility at high temperatures and remains fluid at low temperatures. Their viscosity-temperature characteristics are superior to other isomeric forms of diesters of aromatic dibasic acids.

The most important property of the novel dialkyl diesters of mixtures of isophthalic acid and terephthalic acid of this invention is their thermal stability at high temperatures which make them unusually desirable as base lubricants for aircraft gas turbine lubricating oil compositions. The unusual new synthetic oils, according to the present invention, are characterized by a surprisingly low coke formation when subjected to high temperatures for extended periods of time. They are surprisingly superior in this respect to other synthetic oils commonly employed heretofore in high temperature

2

applications such as the lubrication of aircraft gas turbines.

The dialkyl diesters of mixtures of isophthalic acid and terephthalic acid in accordance with this invention, 5 are illustrated by the following general formula:



in which R<sub>1</sub> is an alkyl group of from 5 to 13 carbon atoms and R<sub>2</sub> is another alkyl group of from 5 to 13 carbon atoms which may be the same as or different from R<sub>1</sub>. Preferably, the R<sub>1</sub> and R<sub>2</sub> alkyl groups are derived by esterifying the mixture of isophthalic acid and terephthalic acid with a mixture of aliphatic alcohols of from 5 to 13 carbon atoms each. Mixtures of from 10 to 90% by weight of each alcohol and from 2 to 5 different kinds are particularly suitable. Still more preferred are esterifying alcohols and alkyl groups derived therefrom within the foregoing description which are mixed, branched chain alcohols of from 6 to 10 carbon atoms with an average of 8 carbon atoms each. Isophthalate and terephthalate mixtures derived from such alcohols are characterized by low volatility and at the same time have less tendency to crystallize at low temperatures.

35 The mixtures of isophthalic acid and terephthalic acid from which the dialkyl diesters of this invention are derived preferably contain from 50 to 99% by weight of isophthalic acid and from 1 to 50% by weight of terephthalic acid. Such proportions occur in the usual mixtures of the two acids derived from isomeric xylenes from common sources such as petroleum fractions or coal tar distillates. Particularly suitable mixtures within the aforementioned proportions are those containing about 85% by weight isophthalic acid and 15% by weight terephthalic acid.

40 Examples of dialkyl diesters of mixed isophthalic acid and terephthalic acid, in accordance with this invention, include n-hexyl 2-ethylbutyl isophthalate and terephthalate having an isophthalate to terephthalate weight ratio of 25 to 75, 2-ethylhexyl isooctyl isophthalate and terephthalate derived from a 50-50 mixture of isophthalic acid and terephthalic acid, 2-ethylhexyl isooctyl diester of a mixture of 85% by weight of isophthalic acid and 15% by weight terephthalic acid, 2-ethylhexyl isooctyl n-octyl mixed diester of 85% by weight isophthalic acid and 15% by weight terephthalic acid, di-2-ethylhexyl diester of a mixture of 85% by weight of isophthalic acid and 15% by weight terephthalic acid, n-amyl n-hexyl isooctyl mixed diester of 85:15 isophthalic acid and terephthalic acid, "Oxo" tridecyl diester of 85:15 isophthalic acid and terephthalic acid, etc.

45 The dialkyl diesters of isophthalic acid and terephthalic acid are conveniently prepared by the reaction of the desired aliphatic alcohols of from 5 to 13 carbon atoms each with the mixture of acids under ordinary esterification conditions. Conventional esterification catalysts such as p-toluenesulfonic acid and heating are desirable to accelerate the reaction.

50 The esterification of the isophthalic acid and terephthalic acid with aliphatic alcohols, as described above, results in dialkyl diesters of three different types for the

isophthalic acid and terephthalic acid. This fact is illustrated by the following equations:



Mixtures of the dialkyl diesters of the above types in which the  $R_1$  and  $R_2$  alkyl groups are different from one another generally have superior physical properties compared to the diesters in which the alkyl groups are alike.

The following examples will serve as further illustrations of the dialkyl diesters of isophthalic acid and ter-

product is decolorized with carbon and topped by distilling at 0.1 mm. mercury pressure to a maximum pot temperature of 200° C. It has an average saponification number of 294 and its equivalent weight estimated from analysis is about 188 compared to a theoretical of 195. The product is then distilled at 0.1 mm. of mercury pressure to a maximum pot temperature of 225° C. The distilled material is clear in appearance and pours slowly at about -55° F.

The physical characteristics of representative examples of the superior new dialkyl diesters of mixtures of isophthalic acid and terephthalic acid of this invention are given in the following table. Also included, for the purpose of comparison, are esters of phthalic acid which is the ortho isomer of isophthalic acid and terephthalic acid.

Table I

| Acid          | Alkyl Groups                  | Viscosity, Centistokes |         |         | Approximate Pour Point, ° F. |
|---------------|-------------------------------|------------------------|---------|---------|------------------------------|
|               |                               | -40° F.                | 100° F. | 210° F. |                              |
| Phthalic      | 2-Ethylhexyl                  | 100,000 extr.          | 29.6    | 4.25    | Cloud at -30.                |
| Phthalic      | Isooctyl                      | 65,000 extr.           | 27.2    | 4.14    | Cloud at -20.                |
| 85-IPA-15-TPA | 2-Ethylhexyl-Isooctyl         | 77,000                 | 33.5    | 4.86    | -55.                         |
| 85-IPA-15-TPA | 2-Ethylhexyl-Isooctyl-n-Octyl | 48,000 extr.           | 28.5    | 4.55    | -60.                         |

ephthalic acid mixtures, according to this invention. Unless otherwise specified, the proportions are given on a weight basis.

#### EXAMPLE I

This example shows the preparation of mixed isoctyl, n-octyl, 2-ethylhexyl ester of a mixture of 85% by weight isophthalic acid and 15% by weight terephthalic acid.

322 g. of 85:15 isophthalic acid and terephthalic acid mixture, 546 g. isoctyl alcohol (75%) 82 g. 2-ethylhexanol (10%) and 109 g. n-octanol (15%) are mixed in a reaction vessel equipped with stirrer, thermometer, water trap and reflux condenser. 5.3 g. sodium bisulfate is added to the mixture. The mixture is heated under reflux conditions for about 16 hours to a maximum pot temperature of about 215° C. under a blanket of nitrogen. 75 ml. water is evolved during this time. This preparation is carried out in duplicate to provide additional product.

The combined products obtained above are washed twice with dilute aqueous sodium carbonate solution and then water until neutral. The products are then treated with 30 g. decolorizing carbon and topped by distilling at 0.1 mm. mercury pressure to a maximum pot temperature of 200° C. to remove unreacted materials. 1,428 g. of bottoms product is obtained. This product is filtered through a column filled with 300 g. of clay to give 1,058 g. of mixed isoctyl, n-octyl, 2-ethylhexyl ester of 85:15 iso- and terephthalic acid which has a clear appearance and pours slowly at about -60° F.

#### EXAMPLE II

The preparation of mixed isoctyl, 2-ethylhexyl diester of a mixture of 85% by weight isophthalic acid and 15% by weight terephthalic acid is shown in this example.

332 g. of 85:15 isophthalic acid and terephthalic acid mixture, 546 g. isoctyl alcohol (75%) and 181 g. 2-ethylhexanol (25%) are added to a reaction vessel provided with stirrer, thermometer, water trap and condenser. 5.3 g. of sodium bisulfate is then added and the mixture heated and refluxed for about 16 hours to a maximum pot temperature of about 215° C. 79 ml. of water is involved.

The product of the above reaction, which is the mixed isoctyl, 2-ethylhexyl ester of 85:15 iso- and terephthalic acid, is washed twice with dilute aqueous sodium carbonate solution and then water until neutral. After this

in the above table the abbreviation "extr." indicates that the viscosity was obtained by extrapolation of the viscosity-temperature curve for the fluid.

From the physical properties of the phthalate esters in the above table, it is readily observed that the mixed dialkyl diesters of isophthalic acid and terephthalic acid are decidedly superior to the corresponding esters of phthalic acid as base lubricants. The viscosity-temperature characteristics are much better, thus providing more effective lubrication over wide temperature ranges. Another advantage of the mixed dialkyl isophthalates and terephthalates lies in their low pour points.

A further illustration of the superior new dialkyl diesters of isophthalic acid and terephthalic acid mixtures of the invention is obtained in an evaluation of the effectiveness of the phthalic esters as aircraft gas turbine lubricants by a number of standard tests on the phthalic ester base lubricants compounded with conventional additives. In these tests the comparison of the results is facilitated by the employment of identically formulated compositions as follows:

|    |                                                              |        |
|----|--------------------------------------------------------------|--------|
| 50 | Ester base stock                                             | 94.378 |
|    | Tricresylphosphate (oiliness additive)                       | 5.0    |
|    | Phenothiazine (oxidation inhibitor)                          | 0.5    |
|    | Quinizarin (metal deactivator)                               | 0.02   |
| 55 | Mixed mono- and didodecyl phosphate octadec- enyl amine salt | 0.1    |
|    | Dimethyl silicone, 60,000 cs. at 25° C. (foam suppressant)   | 0.002  |

60 As mentioned, the tests employed in the evaluations are standard tests known generally to the lubricating art by their descriptions in the table which follows.

The standard coking test involves maintaining the test oil in a bath at a constant level and splashing it against an overhead inclined plate at the temperature indicated for eight hours. The splashing is effected by steel wires on a wheel rotated at a speed of 1,050 r.p.m. as it is partially immersed in the oil. The coking value is the weight of the deposit formed on the underside of the plate during the test period. The description of this coking test is found in gas turbine oil specifications MIL-L-7808C and MIL-L-25336.

The evaporation characteristics of the compositions are determined by placing them in a bomb through which air is passed at a given rate over the fluid. The weight

losses over the period of time at the temperature indicated are reported in terms of percent by weight. This test is the standard ASTM evaporation test D972-51T.

The oxidation and corrosion test involves joining the five metal specimens in the form of a pentagon and immersing them in the oil to be tested. Oxygen is bubbled through the oil at the temperature and for the time indicated and the change in weight of each of the metal specimens is determined.

For the purpose of comparison, the following table also gives illustrated test results on compositions containing base lubricants other than the mixed dialkyl diesters of isophthalic acid and terephthalic acid according to this invention. For example, di(2-ethylhexyl) sebacate is included as illustrative of one of the more commonly used synthetic oil base lubricants. The separate phthalate isomers are also given for comparative purposes.

factorily low level and there is little sludge formed in the compositions.

The novel diesters of mixed isophthalic acid and terephthalic acid have other uses in addition to their application as synthetic oils. Such uses include their employment as plasticizers in compositions where low freezing points are desirable.

I claim:

- Dialkyl diesters of mixtures of isophthalic acid and terephthalic acid in which the alkyl esterifying groups are derived from a mixture of from 2 to 5 aliphatic alcohols of 8 carbon atoms each said mixture containing from 10 to 90% by weight of each alcohol and the mixtures of acid contain from 50 to 99% by weight of isophthalic acid and from 1 to 50% by weight of terephthalic acid.
- Dialkyl diesters of a mixture of 85% by weight of

Table 2

| Ester Type:<br>Alkyl Group.....                                                           | 2-Ethylhexyl, Isooctyl |               |                                            | Di-2-ethylhexyl         | Isooctyl<br>n-octyl 2-<br>ethylhexyl       |
|-------------------------------------------------------------------------------------------|------------------------|---------------|--------------------------------------------|-------------------------|--------------------------------------------|
|                                                                                           | Iso-Phthalate          | Terephthalate | Iso: Ter-<br>ephthalate<br>Ratio,<br>85:15 | Sebacate<br>(Reference) | Iso: Ter-<br>ephthalate<br>Ratio,<br>85:15 |
| Properties:                                                                               |                        |               |                                            |                         |                                            |
| Flash, ° F.                                                                               |                        |               |                                            | 450                     |                                            |
| Fire, ° F.                                                                                |                        |               |                                            | 510                     |                                            |
| Viscosity at 210° F., cs.                                                                 | 4.73                   | 4.87          | 4.77                                       | 3.38                    | 4.56                                       |
| Viscosity at 100° F., cs.                                                                 | 32.74                  | 31.54         | 32.9                                       | 13.1                    | 28.5                                       |
| Viscosity at -40° F., cs.                                                                 | 135,000                | 104,000       | 92,000                                     | 1,700                   | 64,600                                     |
| Neutralization No.                                                                        | 0.31                   | 0.36          | 0.52                                       | 0.90                    | 0.40                                       |
| Oxidation and Corrosion, 72 hours at 347° F.,<br>Metal Wt. Change, Mg./cm. <sup>2</sup> : |                        |               |                                            |                         |                                            |
| Magnesium                                                                                 |                        |               | +0.06                                      | +0.10                   |                                            |
| Steel                                                                                     |                        |               | +0.03                                      | +0.13                   |                                            |
| Silver                                                                                    |                        |               | +0.06                                      | +0.09                   |                                            |
| Aluminum                                                                                  |                        |               | +0.05                                      | +0.02                   |                                            |
| Copper                                                                                    |                        |               | +0.09                                      | +0.45                   |                                            |
| Used Oil:                                                                                 |                        |               |                                            |                         |                                            |
| Percent change in 100° F. vis.                                                            |                        |               | +4.66                                      | +1.5                    |                                            |
| Change in Neutralization No.                                                              |                        |               | +0.1                                       | +1.09                   |                                            |
| Percent pentane insolubles.                                                               |                        |               | 0.42                                       | 0.24                    |                                            |
| Coking, 8 hours at 600° F., mg.                                                           |                        |               |                                            | 15                      |                                            |
| Coking, 8 hours at 700° F., mg.                                                           | 1,560                  | 984           | 804                                        | 3,600                   | 11,900                                     |
| Used Oil from Sump:                                                                       |                        |               |                                            |                         |                                            |
| Percent change in 100° F. vis.                                                            | +16.7                  | +21.4         | +11.7                                      | +24.1                   |                                            |
| Change in Neutralization No.                                                              | +2.6                   | +2.3          | +3.0                                       | 0.0                     | +2.5                                       |
| Percent pentane insolubles.                                                               | 0.34                   | 0.35          | 0.24                                       | 0.05                    | 0.46                                       |
| Evaporation, 615 hours at 400° F., Percent                                                | 16                     | 13            | 15                                         | 10-14                   | 14                                         |

<sup>1</sup> + Coke value equivalent to an 8-hour test. Test terminated before 8 hours.

The above test results show that the mixed dialkyl diesters of isophthalic acid and terephthalic acid are outstanding synthetic oil base fluids for aircraft gas turbine lubricating oils. They possess excellent thermal stability at high temperatures as indicated by their low coke formation. In this very important characteristic for gas turbine lubricants, it can be seen at once from the above results that the mixed dialkyl diesters of isophthalic acid and terephthalic acid give lubricant compositions which are decidedly superior to similar compositions containing the widely used di(2-ethylhexyl) sebacate as base lubricant. The coking characteristics of the mixed isophthalates and terephthalates of the invention are also surprisingly superior to the separate isomeric phthalates.

The above table also shows that the mixed isophthalate and terephthalate base gas turbine lubricant compositions of the invention possess excellent volatility characteristics which prevent undue consumption of the lubricant compositions at high altitudes and high temperatures. The mixed isophthalates and terephthalates are also fluid at unusually low temperatures and have good viscosity temperature characteristics which make them suitable as lubricants throughout wide temperature ranges.

The compositions of the invention are also shown to be unusually resistant to oxidation and formation of corrosive products at high temperatures. The corrosion of all types of metals in the tests is maintained at a satis-

isophthalic acid and 15% by weight of terephthalic acid in which the alkyl esterifying groups are derived from a mixture of from 2 to 5 aliphatic alcohols of 8 carbon atoms each, said mixture of alcohols containing from 10 to 90% by weight of each alcohol.

55 3. 2-ethylhexyl isoctyl diester of a mixture of 85% by weight isophthalic acid and 15% by weight terephthalic acid in which the 2-ethylhexyl and isoctyl esterifying groups are derived from a mixture consisting of 25% by weight of 2-ethylhexyl alcohol and 75% by weight of isoctyl alcohol.

55 4. Mixed isoctyl, n-octyl and 2-ethylhexyl diesters of a mixture of 85% by weight isophthalic acid and 15% by weight terephthalic acid in which the esterifying groups are derived from a mixture consisting of 75% by weight of isoctyl alcohol, 15% by weight of n-octyl alcohol and 10% by weight of 2-ethylhexyl alcohol.

References Cited in the file of this patent

UNITED STATES PATENTS

- |              |                    |                |
|--------------|--------------------|----------------|
| 70 2,610,205 | Trigg et al. ----- | Sept. 9, 1952  |
| 2,628,207    | Smith et al. ----- | Feb. 10, 1953  |
| 2,650,908    | Beears -----       | Sept. 1, 1953  |
| 2,653,165    | Levine -----       | Sept. 22, 1953 |
| 2,656,377    | Pino -----         | Oct. 20, 1953  |
| 2,802,860    | Stack et al. ----- | Aug. 13, 1957  |
| 75 2,809,208 | Miller -----       | Oct. 8, 1957   |